

# UNITED STATES PATENT OFFICE.

WILLIAM C. SWIFT, OF CAMBRIDGE, MASSACHUSETTS, ASSIGNOR TO STANDARD WOVEN FABRIC COMPANY, OF WALPOLE, MASSACHUSETTS, A CORPORATION OF MASSACHUSETTS.

## PROCESS OF MAKING FRICTION FACINGS.

1,426,842.

Specification of Letters Patent. Patented Aug. 22, 1922.

No Drawing.

Application filed November 26, 1918. Serial No. 264,245.

To all whom it may concern:

Be it known that I, WILLIAM C. SWIFT, a citizen of the United States, residing at Cambridge, in the county of Middlesex and State of Massachusetts, have invented certain Improvements in Processes of Making Friction Facings, of which the following description is a specification.

This invention relates to friction facings, such as clutch rings and brake linings. As is well understood by those familiar with the various types of clutches and brakes, it is the usual practise to line or face a brake or clutch element with a material capable of resisting wear, giving the desired co-efficient of friction, and adapted to resist the relatively high temperatures which are created between the elements of the clutch or brake under certain conditions of service. Particularly important examples of this practise are found in the clutches and brakes used in motor vehicles.

At the present time the more usual clutch facings and brake linings are made from a heavy asbestos fabric, the yarn from which the fabric is woven usually being reinforced by a fine wire and the fabric being "doped," that is, impregnated with a binder, which usually is cured by heat and which serves to bind together the fibres of asbestos or other material used in the fabric and to consolidate the material and enable it better to resist wear. The co-efficient of friction of the facing also depends largely upon the nature of this dope, or impregnating compound, and the curing treatment which it undergoes.

It is obvious that the spinning and weaving operations necessitate the use of a relatively long fibre asbestos; and while it was proposed a number of years ago to make friction facings of this character from short fibre asbestos by processes that would eliminate the necessity for the spinning and weaving operations, such facings have never been used to any substantial extent until very recently, when the extraordinary rise occurred in the price of crude or long fibre asbestos. Of the various processes heretofore suggested for making these facings from short asbestos fibre, the most successful process now in use, of which I am aware, consists essentially in forming an asbestos board or sheet, usually in a paper making machine, and then impregnating the sheet stock so

formed with a binding material, dieing out 55 rings or other facing parts of the desired shape and dimensions, from this sheet stock, and baking and pressing the parts so dieed out to cure the binder and consolidate the facing. In some instances the facings are 60 dieed out before the impregnating operation is performed.

While friction facings manufactured in the manner just described have met with some degree of success, it has been impracticable 65 to produce commercially a facing of uniform or homogenous character, due chiefly to the difficulty of uniformly impregnating the facing with the binding material. It is obvious that since the binder performs a very im- 70 portant function in facings of this character, the failure to realize a uniform impregnation of the material will result in varying the wearing qualities and co-efficient friction of the facing at different 75 points therein as its surface becomes worn away. The present invention is directed to the improvement of the processes of making unwoven friction facings of the character above described and it aims particu- 80 larly to devise a process which will produce facings of a more uniform and homogeneous character than those heretofore proposed, and in which a uniform impregnation of the facing will be effected. 85

The nature of the invention will be readily understood from the following description and the novel features of the invention will be pointed out more particularly in the appended claims. 90

According to the present invention the materials that form the body of the facing, and which will vary in character and proportions according to the formulas of different manufacturers, are all placed in a 95 beater or an agitator and mixed with a relatively large quantity of liquid. Whether or not a beater is used will depend upon the nature of the materials and the condition in which it is desired to bring them together. 100 If the materials are relatively coarse it may be necessary to run them through a beater before they are brought into the agitator. The short fiber asbestos, however, comes in a very finely divided condition and usually 105 the other materials that go into a facing of this character are in the state in which they are purchased in the open market in a

pulverized, or at least in a very finely divided, condition so that it is merely necessary to use an agitator to effect the initial mixing of the ingredients. Assuming, for 5 instance, that the clutch facing is to be made from 55%, by weight, of short fibre asbestos, 40% of Portland cement and 5% of binder, these materials would all be brought together in a finely divided condition and 10 mixed with a large quantity of a solvent for the binder, this solvent being used in the present process in place of the water that is ordinarily used in the paper making process. A crude form of asphaltum is very 15 commonly used as a binder and is dissolved in naphtha, gasoline, or benzol preparatory to performing the impregnating operation. Consequently, when this binder is used, a solvent for it is employed as the liquid in 20 which the finely divided materials are held in suspension during the formation of the sheet stock. This mixture of liquid solvent and the materials held in suspension thereby are run through a paper making machine, 25 preferably of the cylinder type in which a sheet of the required thickness is built up. As is well understood by those skilled in this art, the machine strains out enough of the solid matter to form a very thin flimsy sheet 30 and this sheet is transferred to a cylinder on which it is wound to build up a board or sheet of the required thickness. The liquid, after passing through the screen and depositing the solid material carried thereby, 35 or at any rate a very large percentage of it, is collected in suitable receptacles and returned to the agitator where it is again mixed with raw materials in readiness to repeat the process.

40 It is obvious that this process produces a sheet stock in which an absolutely uniform impregnation of the stock with the binder is effected. That is, the binder being present in the form of a solution or held in suspension 45 in the liquid which also holds the other materials in suspension, ensures a very intimate contact of the binder with the fibers and particles of materials that make up the sheet. Consequently, when a sheet of the 50 required thickness has been built up on the cylinder of the paper machine and is removed from this cylinder in the usual way, the binder is distributed uniformly through the entire depth of the sheet.

55 Preferably facings of the desired form are died out of this sheet stock while it is still damp and before the cement, in case such material is used, has had an opportunity to set. These facings are then pressed and 60 baked. In the case of clutch rings, for which the present process is particularly adapted, the rings after being died out may be stacked on suitable arbors and separated by thin sheet metal disks or rings while the 65 baking operation is being performed. In

any event, the baking operation melts the particles of binder which are distributed uniformly throughout the entire body of the ring and cures this binder, driving out the volatile matter and leaving the ring in a 70 hard, firm and dry condition.

It is obvious that the treatment after the facing has been formed may vary with the requirements and practices of different manufacturers and may follow that usually employed at the present time subsequent to the impregnation step. But the present invention is advantageous in any of these cases in effecting a uniform impregnation of the product, avoiding the necessity for a separate doping or impregnating operation and ensuring an absolutely homogeneous facing.

It will be understood that the process herein described is by no means limited to use with the specific formula above suggested, 85 that formula being proposed merely by way of illustration, and that the distinguishing feature of this process is that the impregnating process is united with the paper making or sheet forming process by using, for the 90 liquid necessary in the sheet forming process, one in which the binder is soluble, or which at least holds the binder in suspension in a finely divided condition.

As examples of other formulas, it may be 95 stated that for some uses the friction facing is made entirely of asbestos fibre with a binder, while in other cases a substantial percentage of Portland cement or of some inert filler, such as clay, kaolin, or the like, 100 is employed. Various materials are employed as binders besides the crude asphaltum above mentioned, for instance, bakelite, mineral waxes, and in some cases, a vegetable binder. The nature of the solvent employed obviously depends upon the 105 nature of the binder used, and the quantity of solvent will depend more upon mechanical than chemical conditions. That is, the percentage of solid matter carried by the 110 liquid as it goes through the paper making machine is very small, and the quantity of liquid employed will be controlled by the requirements of the paper making or sheet forming process rather than by the necessity 115 for dissolving the binder.

This process completely obviates the very embarrassing difficulty of properly impregnating the facing material or stock which has been experienced heretofore, and facings 120 made according to this process are even superior in wearing properties than the fabric facings heretofore more commonly used. When solvents of a very volatile nature are used, such as gasoline, benzol, and the like, 125 the solvent vapors that escape during the process of manufacture may be recovered by processes similar to those used for this purpose in other arts, as, for instance, in the rubber coating industries.

What is claimed as new, is:—

1. The process of making blank stock for friction facings which consists in mixing the facing materials, including asbestos fibre and a binder, substantially insoluble in water, with a relatively large quantity of liquid solvent for the binder to enable said liquid to hold the materials in suspension, and then straining out a sufficient quantity of the solid matter from the mixture to form a blank of suitable form and thickness, whereby said blank will be uniformly impregnated with the binder.
2. The process of making blank stock for friction facings which consists in mixing the facing materials, including asbestos fibre and a binder, with a relatively large quantity of liquid hydrocarbon in which the binder is soluble to enable said liquid to hold the materials in suspension, then running the mixture through a paper making machine and forming therein a sheet of the required thickness, whereby said sheet will be uniformly impregnated with the binder.
3. The process of forming friction facing stock from finely divided materials including asbestos fibre and a binder substantially insoluble in water, which consists in utilizing the paper making process to bring said materials into a sheet form, and using a liquid solvent for said binder to hold said

materials in suspension while the sheet is being formed, whereby said sheet will be uniformly impregnated with the binder.

4. The process of forming friction facings from finely divided materials including asbestos and a binder, which consists in utilizing the paper making process to bring said materials into the form of a facing blank, and using a liquid hydrocarbon solvent for said binder to hold said materials in suspension while said blank is being formed, whereby said blank will be uniformly impregnated with the binder, shaping said blank to the desired form and then baking the article so shaped to cure the binder and harden the facing.

5. The process of forming friction facing stock from finely divided materials including a binder substantially insoluble in water, which consists in utilizing the paper making process to bring said materials into a sheet form, and using a liquid solvent for said binder to hold said materials in suspension while the sheet is being formed, cutting facings of the desired form from said sheet, and then baking the facings to cure the binder and harden the facing.

In testimony whereof I have signed my name to this specification.

WILLIAM C. SWIFT.